

## UNITED STATES PATENT OFFICE

RALPH R. CURRY, OF TARENTUM, PENNSYLVANIA, ASSIGNOR TO ALLEGHENY STEEL COMPANY, OF BRACKENRIDGE, PENNSYLVANIA, A CORPORATION OF PENNSYLVANIA

## METHOD OF MAKING DUCTILE HIGH-SILICON-STEEL SHEETS

No Drawing.

Application filed July 27, 1927. Serial No. 208,897.

This invention relates to the manufacture of silicon steel sheets such as used in the construction of certain portions of electrical apparatus including the cores for transformers.

5 Silicon steel now used in sheet form in the construction of cores for transformers and for other parts of electrical apparatus has a silicon content, as a general rule, of from 1% to 4½% depending upon the electrical 10 properties which are required in such sheets. The grades having a high silicon content, as for instance, of from 3½% to 4% are almost entirely used in the construction of transformer cores because of their low hysteresis 15 losses. Generally speaking, it is found that the higher the silicon content, the lower will be the hysteresis loss.

Silicon steel having a silicon content in excess of 4% when rolled into light gauge sheets 20 and annealed is, as a general thing, so brittle as to cause the manufacturers of such sheets to effect a compromise, in other words, to manufacture a silicon steel in which a portion of its electrical value is sacrificed in favor 25 of its ductility or malleability with the result that silicon steel having a silicon content in excess of 4% is seldom rolled into light gauge sheets for use in the manufacture of electrical apparatus.

25 The practice of effecting this compromise has limited the manufacturers of such sheets to silicon steel having a maximum silicon content just short of that from which a considerable advantage would be gained in electrical 35 quality, especially where the sheets are to be used in equipment operated at high flux densities.

For example, a steel having a silicon content of 4% is not as a general rule better than 40 a steel having a silicon content of 3.75%, but a steel having a silicon content of 4.25% is very materially better and will give materially better results electrically than one having a silicon content of but 4% especially 45 if tested to high densities.

Under the ordinary methods of manufacture, a silicon steel having a silicon content of 4.25% or any silicon content in excess of 4% is so brittle that its conversion into sheets 50 of proper thickness or gauge entails a con-

siderable loss, a large percentage being bound to fail to meet the commercial standards of ductility or malleability.

An object of this invention is to improve the present methods of manufacturing silicon 55 steel sheets so that sheets having a silicon content in excess of 4% may be readily rolled into relatively thin sheets without the losses now encountered because of the lack of ductility or malleability of the sheets made under the 60 present methods.

I have discovered that by a slight change or modification of the methods now utilized in the making of light gauge sheets of the higher silicon content steels I am able to reduce the brittleness to an extent that will permit the sheets to pass the commercial standard of ductility or malleability and because of the higher silicon content an improvement 65 in the electrical qualities is obtained. 70

In the ordinary process of making silicon steel sheets for use in electrical apparatus the ingot is rolled into sheet bars of a thickness that will give the required length for the gauge of sheets being produced. These bars 75 are then heated to a rolling temperature and given a number of operations until the final length and gauge of the sheets is obtained.

I have found that if, after the bars have attained the rolling temperature, they are 80 held at that temperature for some time or soaked as the steel maker terms it, I can produce sheets that are considerably more ductile than those produced in the regular way. In fact, by raising the sheet bars of silicon steel 85 having a silicon content of 4.25% to rolling temperature and then holding them at that temperature for from 1 to 4 hours and then converting these heated bars into sheets in the regular way, I obtain ductile sheets of 90 silicon steel even though the silicon content is as high as 4.50%.

The improvement in the ductility or malleability of such sheets is so marked over those produced in the regular way that there 95 is practically no loss for this reason.

This soaking of the sheet bars apparently permits the crystals or grains of the steel to adjust themselves in a manner which in the subsequent rolling to light gauge produces 100

an arrangement of crystals or grains which improves the ductility of the sheets.

I have found that an excessive length of time for this soaking step is not necessary. From one to four hours is usually sufficient to obtain the necessary ductility or malleability in all cases. Sheet bars which I have soaked for eight hours for instance, do not give measurably softer nor more ductile sheets than those which have been soaked for only two hours. The length of time of soaking may be somewhat varied to meet different requirements as to ductility or malleability, but in most cases a soaking at rolling temperature of about two hours is found sufficient.

Having thus described my invention, what I claim is:—

1. That step in the art of rolling silicon steel sheets for use in electrical apparatus, which consists in rolling sheet bars in slowly raising the temperature of such bars to rolling temperature and in holding the same at that temperature for at least one hour whereupon ductile relatively thin sheets may be rolled therefrom.

2. That step in the art of rolling silicon steel sheets, which consists in rolling sheet bars from such metal in slowly raising the temperature of such bars to rolling temperature, in holding said bars at that temperature for at least one hour and then in rolling sheets therefrom.

3. That step in the art of rolling silicon steel sheets, which consists in rolling sheet bars from such metal in slowly raising the temperature of such bars to rolling temperature, in holding said bars at that temperature for about one hour and then in rolling sheets therefrom.

4. The method of making ductile silicon steel sheets having a relatively high silicon content, which consists in forming an ingot of such silicon steel, in rolling the same into sheet bars, in cutting said bars into suitable lengths, in raising such cut bars to rolling temperature, in holding the same at substantially this temperature for at least one hour, and then in converting said bars into sheets of the required gauge.

5. The method of making ductile silicon steel sheets having a relatively high silicon content, which consists in forming an ingot of such silicon steel, in rolling the same into sheet bars, in cutting the bars into suitable lengths, in raising such cut bars to rolling temperature, in holding the same at substantially this temperature for at least one hour to cause a readjustment of the grain thereof, and then in converting said bars into sheets of the required gauge.

In testimony whereof, I have hereunto subscribed my name this 22nd day of July, 1927.

RALPH R. CURRY.